# EUROPEAN PATENT SPECIFICATION

(11) **EP 0 151 825 B1**
(45) Date of publication and mention of the grant of the patent: **02.11.1989**
(21) Application number: 84201821.0
(22) Date of filing: 10.12.1984
(51) Int. Cl.: C10M 117/04

(54) **Process for the continuous manufacture of a lubricating grease**
Verfahren zum kontinuierlichen Herstellen von Schmierfett
Procédé pour fabriquer en continu une graisse lubrifiante

(30) Priority: 04.01.1984 GB 8400073
(43) Date of publication of application: 21.08.1985
(73) Proprietor: SHELL INTERNATIONALE RESEARCH MAATSCHAPPIJ B.V., 2596 HR Den Haag (NL)
(72) Inventor: Coleclough, Norman, Cheshire CH1 3SH (GB); MacPhail, Alexander Colquhoun Barr, Cheshire CH1 3SH (GB); Roberts, Kenneth Edward, Cheshire CH1 3SH (GB)
(74) Representative: Aalbers, Onno

(56) References cited:
- EP-A- 0 072 184
- GB-A- 579 847
- GB-A- 1 508 281
- GB-A- 2 086 249
- GB-A- 2 127 430
- US-A- 4 315 825

## Description

This invention relates to a process for the continuous manufacture of a lubricating grease and in particular of a base grease which serves as a basis for the manufacture of a wide variety of lubricating grease formulations containing one or more additives. By first making a base grease a great flexibility is obtained in making a great variety of grease formulations using the same grease manufacturing basic unit.

From European patent application 0072184 a process for the continuous manufacture of a lubricating grease, which process shows a great flexibility, is already known. According to this process a rotating screw process unit is used.

It has now been found that such processes, which enable the manufacture of a great variety of greases, such as the greases described in said European patent application, can be carried out in a simpler way without the use of moving parts, namely by using motionless mixers, which are readily commercially available.

Therefore the present invention relates to a process for the continuous manufacture of a lubricating grease comprising blending feed materials and lubricating oil and pumping the resulting blend through at least one motionless mixer which is heated to such a temperature that soap formation takes place and a resultant grease is formed.

Suitable feed materials are the usual thickening or gelling agents which in the case of soaps are often made in situ in at least part of the lubricating oil from saponifiable material, saponification agents and optionally complexing agents.

Suitable saponifiable materials are long chain fatty esters, especially glycerides, in particular where the fatty group contains a hydroxy radical, such as ricinoleyl (castor oil) or hydrogenated ricinoleyl (hydrogenated castor oil).

Another method of soap formation is to neutralize fatty acids or hydroxy fatty acids in mineral oil with alkali metal or alkaline earth metal hydroxides (or mixtures of both) or hydrates thereof - in particular lithium hydroxide monohydrate (LiOH.H₂0). Alternatively hydrogenated fatty acids or hydrogenated hydroxy fatty acids are commonly used in the neutralization.

Suitable saponification agents are alkali metal or alkaline earth metal hydroxides (or mixtures of both), in particular lithium hydroxide, or hydrates thereof. Therefore, the feed materials preferably comprise
a) hydrogenated castor oil (HCO) and lithium hydroxide or lithium hydroxide monohydrate;
b) HCO and lithium hydroxide (or monohydrate) or calcium hydroxide;
c) Hydrogenated castor oil -fatty acid (HCOFA) and lithium hydroxide or lithium hydroxide monohydrate; and/or
d) HCOFA and lithium hydroxide (or monohydrate) or calcium hydroxide.

Suitable complexing agents are short chain fatty acids, such as acetic acid, dicarboxylic acids, such as azelaic acid, hydroxy aromatic acids such as salicyclic acid, boric acid, aluminium compounds, etc. If such complexing agents are used the proportion of saponification agents is usually increased with about the stoichiometric quantity of the complexing agent.

Other suitable thickening agents are clays, including coated clays, silica gels, polymers, polyureas, carbon black, dyes, etc.

Suitable lubricating oils are mineral oils, including hydrogenated mineral oils, synthetic oils, such as ester oils, polyolefin oils, silicon oils, phosphate esters, polyphenyl ethers, etc. Suitable mineral lubricating oils include HVI, paraffinic MVI, naphthenic MVI and LVI oils.

To the base greases may be added additional lubricating oil and additives, such as antioxidants, antirust, anti-wear and extreme pressure agents, pour point depressants, metal deactivators etc.

Suitable laboratory-type motionless or static mixers have the form of a cylinder or tube having a length of 65.5 to 66.5 cm and a diameter of 3.3 to 3.6 cm. They are provided with an insulated heating jacket, using e.g. electric tape having a heating capacity of e.g. 400 watt per mixer, or a heating medium as the heating source. The inside of the cylinder is provided with e.g. corrugated plates, perforated plates, intermeshing and intersecting bars and similar fixed mechanical obstacles causing mixing and heat exchange. A suitable motionless mixer containing perforated plates is described in e.g. GB-A-2086249, but other types may be used as well.

Suitable mixers are: the Sulzer motionless mixer SMX type which is 655 mm long x 36 mm internal diameter and the Sulzer motionless heat exchanger SMXL type which is 665 mm long x 32.8 mm internal diameter.

For commercial production the sizes of the mixers require scaling up.

According to the present process the base grease-making ingredients are preferably blended at room temperature in a container from which they are pumped through at least one motionless mixer, preferably several motionless mixers, preferably longitudinally connected. They may also be, or additionally be, connected in a parallel manner.

The average velocity of the mixture in the mixers may be 3 kg to 50 kg/h, preferably 7 to 30 kg/h, the flow preferably being laminar.

The pressure at the entrance of the first mixer may be between 1 and 30 bar, preferably between 1 and 15 bar.

The mixers are heated to a suitable high temperature, e.g. at least 120°C, preferably between 120 and 250°C, preferably up to a maximum temperature between 180 and 230°C, so that a grease structure is formed on cooling. Preferably the temperature of each of the heated mixers is higher than that of the preceding mixer and so on.

Thermocouples may be placed between the mixers for temperature control.

If desired part of the finished grease may be recycled. Also the pump at the entrance of the first mixer may be provided with a recycling circuit.

The subsequent removal of water can be accomplished by simply dumping the resulting grease in an open vessel, whereafter any further lubricating oil and any desired additives can be added.

Due to condensation some water may be present in the open vessel. If required complete dehydration may be accomplished using conventional flash vacuum equipment.

Preferably the base grease together with additional lubricating oil and additives is pumped through a heat exchanger tube for mixing and cooling to obtain the desired consistency.

Homogenisation of the grease, if necessary, is carried out using e.g. a Manton Gaulin homogeniser at 3000 psig (20.7 MPa), a mill or a rolling device etc.

The invention is illustrated by the following Examples.

### Example 1

1.3 kg feed containing: 12 %w hydrogenated castor oil, 1.7 %w LiOH.H₂0, 86.3 %w mineral lubricating oil (HVI, viscosity 10.7-11.8 cSt at 100°C, VI = 96 (min), and 3 %2 (= 39 g) water is mixed at room temperature for at least 10 minutes in a container and then pumped at a flow rate of 8.3 kg/h once through a series of 4 Sulzer motionless mixers (each unit containing 2 mixing elements) which are beforehand adjusted to temperatures of 130,170,190 and 230°C, respectively, by 4 200 watt electric heaters per mixer.

The finished grease is obtained at the outlet and cooled in a jacketed SULZER MONOTUBE HEAT EXCHANGER which consists of 2 units each 1540 mm long x 32.8 mm internal diameter. Each unit contains 1 SMXL type heat exchanger. The unworked/worked penetration at 25°C was 262/273 dmm (ASTM D217-82). (1 dmm corresponds with 0.1 mm) and the dropping point was 197°C. (Worked penetration is the penetration at 25°C after 60 double strokes in a standard grease worker).

The first two Sulzer mixers were of the type SMX DN32, having a length of 655 mm and an internal diameter of 36 mm and the last two were of the type SMXL DN32 (heat exchanger type for boosting the heat transfer during warming up of the viscous mixture), having a length of 665 mm and an internal diameter of 32.8 mm.

Subsequently the water present in the grease was flashed off.

Examples 2-6 are carried out in the arrangement of Example 1, but the flow rate is changed, resulting in different outlet temperatures, penetrations and dropping points (see Table A).

## Claims

1. A process for the continuous manufacture of a lubricating grease comprising blending feed materials and lubricating oil and pumping the resulting blend through at least one motionless mixer which is heated to such a temperature that soap formation takes place and a resultant grease is formed.

2. A process according to claim 1, wherein the blending of feed materials and lubricating oil is carried out at room temperature.

3. A process according to claim 1 or 2, wherein the feed materials comprise
a) hydrogenated castor oil (HCO) and lithium hydroxide or lithium hydroxide monohydrate;
b) HCO and lithium hydroxide (or monohydrate) or calcium hydroxide;
c) Hydrogenated castor oil fatty acid (HCOFA) and lithium hydroxide or lithium hydroxide monohydrate; and/or
d) HCOFA and lithium hydroxide (or monohydrate) or calcium hydroxide.

4. A process according to any one of claims 1-3, wherein a series of heated motionless mixers is used, each mixer having a higher temperature than the preceding one.

5. A process according to any one of claims 1-4, wherein the motionless mixers have perforated plates.

6. A process according to any one of claims 1-5, wherein the mixers are heated to a temperature between 120 and 250°C.

7. A process according to any one of claims 1-6, wherein the resulting grease is cooled in a heat exchanger tube.

8. A process according to any one of claims 1-7, wherein to the resulting grease additional lubricating oil and additives are added.

## Patentansprüche

1. Ein Verfahren zur kontinuierlichen Herstellung eines Schmierfettes umfassend das Vermischen von Ausgangsmaterialien und Schmieröl und das Pumpen der erhaltenen Mischung durch mindestens einen statischen Mischer, welcher auf eine solche Temperatur erhitzt ist, daß die Seifenbildung stattfindet und sich ein entsprechendes Fett bildet.

2. Ein Verfahren gemäß Anspruch 1, in welchem das Mischen von Ausgangsmaterialien und Schmieröl bei Umgebungstemperatur durchgeführt wird.

. 3. Ein Verfahren gemäß Anspruch 1 oder 2, in welchem die Ausgangsmaterialien die nachstehenden Kombinationen umfassen:
a) Hydriertes Ricinusöl (HCO) und und Lithiumhydroxid oder Lithiumhydroxid-Monohydrat;
b) HCO und Lithiumhydroxid (oder dessen Monohydrat) oder Calciumhydroxid;
c) Hydrierte Ricinusöl-Fettsäure (HCOFA) und Lithiumhydroxid oder Lithiumhydroxid-Monohydrat; und/oder
d) HCOFA und Lithiumhydroxid (oder dessen Monohydrat) oder Calciumhydroxid.

4. Ein Verfahren gemäß irgendeinem der Ansprüche 1 bis 3, in welchem eine Serie von beheizten statischen Mischern verwendet wird und jeder Mischer eine höhere Temperatur als der vorhergehende aufweist.

5. Ein Verfahren gemäß irgendeinem der Ansprüche 1 bis 4, in welchem die statischen Mischer perforierte Platten aufweisen.

6. Ein Verfahren gemäß irgendeinem der Ansprüche 1 bis 5, in welchem die Mischer auf eine Temperatur zwischen 120 und 250°C erhitzt werden.

7. Ein Verfahren gemäß irgendeinem der Ansprüche 1 bis 6, in welchem das gebildetet Fett in einem Wärmeaustauscherrohr abgekühlt wird.

8. Ein Verfahren gemäß irgendeinem der Ansprüche 1 bis 7, in welchem zu dem gebildeten Fett zusätzlich Schmieröl und Zusatzstoffe zugesetzt werden.

## Revendications

1. Procédé pour la fabrication en continu d'une graisse lubrifiante qui comprend le mélange de matériaux d'alimentation et d'une huile lubrifiante et le pompage du mélange résultant à travers au moins un mélangeur sans mouvement qui est chauffé à une température telle qu'il se produit une formation de savon et qu'il se forme une graisse résultante.

2. Procédé selon la revendication 1, dans lequel on effectue le mélange des matériaux d'alimentation et de l'huile lubrifiante à la température ambiante.

3. Procédé selon la revendication 1 ou 2, dans lequel les matériaux d'alimentation comprennent
a) de l'huile de ricin hydrogénée (HRH) et de l'hydroxyde de lithium ou de l'hydroxyde de lithium monohydraté,
b) HRH et de l'hydroxyde de lithium (ou son monohydrate) ou de l'hydroxyde de calcium;
c) un acide gras d'huile de ricin hydrogénée (AGHRH) et de l'hydroxyde de lithium ou de l'hydroxyde de lithium monohydraté; et/ou
d) AGHRH et de l'hydroxyde de lithium (ou son monohydrate) ou de l'hydroxyde de calcium.

4. Procédé selon l'une quelconque des revendications 1 à 3, dans lequel on utilise une série de mélangeurs chauffés sans mouvement, chaque mélangeur ayant une température supérieure à celle du précédent.

5. Procédé selon l'une quelconque des revendications 1 à 4, dans lequel les mélangeurs sans mouvement ont des plaques perforées.

6. Procédé selon l'une quelconque des revendications 1 à 5, dans lequel les mélangeurs sont chauffés à une température comprise entre 120 et 250°C.

7. Procédé selon l'une quelconque des revendications 1 à 6, dans lequel on refroidit la graisse résultante dans un tube échangeur de chaleur.

8. Procédé selon l'une quelconque des revendications 1 à 7, dans lequel on ajoute à la graisse résultante, une huile lubrifiante et des additifs supplémentaires.
